

# UNITED STATES PATENT OFFICE.

HENRY STANLEY TIRRELL, OF BROCKTON, MASSACHUSETTS, ASSIGNOR TO L. Q. WHITE SHOE COMPANY, OF BRIDGEWATER, MASSACHUSETTS, A CORPORATION OF MASSACHUSETTS.

## SHOE-FILLER COMPOSITION.

1,258,272.

Specification of Letters Patent. Patented Mar. 5, 1918.

No Drawing.

Application filed March 10, 1916. Serial No. 83,430.

*To all whom it may concern:*

Be it known that I, HENRY STANLEY TIRRELL, a citizen of the United States, residing at Brockton, county of Plymouth, State of Massachusetts, have invented an Improvement in Shoe-Filler Compositions, of which the following description is a specification.

This invention relates to a shoe bottom filler, such as is used in the manufacture of 10 welt shoes for filling the cavity in the bottom of the shoe, and particularly to shoe filler compounds of that class which include an inert granular material, such as ground cork, ground leather, sawdust, etc., mixed 15 with a binder material. The object of the invention is to provide a marketable shoe bottom filler of this type which can be inexpensively and economically manufactured, which will be permanently pliable at 20 all ordinary temperatures of use, which is water-proof, and which is low-melting, quick-setting and easily workable at a temperature obtained in a steam-jacketed kettle.

I propose to use asphalt as the principal 25 ingredient of the binder in my improved shoe filler compound and preferably the natural asphalt such as is obtained from the solid bitumens produced on the island of Trinidad, or in Venezuela, or Oklahoma, and 30 similar places. This asphalt in its natural condition is brittle when cold, although it will readily soften under moderate temperatures. When soft, it is sticky, tacky, tough and tenacious. In order to provide a binder 35 which will not be brittle at ordinary temperatures as the natural asphalt is, but which instead will be permanently pliable and strongly adherent, I propose to temper the asphalt with a mineral wax or a mineral 40 oil, preferably a paraffin wax or paraffin oil. I find that by mixing a mineral oil or mineral wax of this nature with the asphalt, a binder will be produced which will be permanently pliable and strongly adherent 45 and which makes an excellent binder for use in shoe filler compositions. In making the binder the asphalt in its natural condition is heated until it is liquid and then the requisite amount of mineral wax or 50 mineral oil is added and mixed therewith. This produces a binder which is free-flowing at temperatures of 180° or 190° F. and which at this temperature can be readily 55 mixed with the inert filler material, such as ground cork, ground leather, sawdust, etc.

While I find that asphalt tempered with a mineral oil or mineral wax makes an excellent binder for shoe filler composition, yet I do not wish to be limited to the use 60 of mineral oil or mineral wax for this purpose as my invention is intended to cover a shoe filler composition having a binder formed from asphalt which is tempered by mixing therewith any suitable ingredient 65 which will reduce the binder to the desired condition of permanent pliability and which will give to the binder the quick-setting quality.

The characteristic of asphalt varies somewhat, depending upon the particular location from which it is derived and, therefore, the amount of wax or oil necessary to properly temper it may vary. I find that a suitable binder for a filler compound can 70 be made by taking approximately 75 pounds of asphalt having a melting point of approximately 115° F. and 25 pounds of paraffin wax having a melting point of approximately 125° F. and heating these ingredients until they are melted, and then 75 mixing them together. To every 70 pounds of this liquid is added approximately 30 pounds of some inert filler material, such as ground cork, ground leather, sawdust, etc., and the whole is thoroughly mixed to 80 produce a homogeneous mass. A compound made in this way will be permanently pliable, will melt at from 110° F. to 120° F., and thus may be readily softened in a steam-jacketed kettle and when thus softened it 85 can be easily spread onto the bottom of a shoe. It is tenacious and sticky and will thus readily stick to the shoe, and it has quick-setting properties, so that when applied to the shoe it will quickly set, thus permitting subsequent operations to be performed on the shoe without delay. Moreover, although it is pliable so that it will 90 easily bend without breaking or cracking, yet it is stable and will not shift in position 95 in the shoe while the latter is being used.

While I have described herein a particular formula, yet the proportions may be varied, depending on the character of the 100 asphalt and tempering component used.

105

I claim:

1. A shoe bottom filler composed of finely comminuted inert material tenaciously held together by a binder composed of asphalt tempered with a paraffin material to produce a permanently-pliable mass.
2. A shoe bottom filler comprising comminuted inert material tenaciously held together by a permanently-pliable binder consisting of asphalt tempered with a paraffin material to produce a compound melting at 110° F. to 120° F.
3. A shoe bottom filler comprising com-

minuted inert material tenaciously held together by a permanently-pliable binder made up of approximately seventy-five per cent. of asphalt.

4. A binder for shoe filler composition comprising an asphalt tempered with paraffin material to produce a compound melting at a temperature of from 110° F. to 120° F.

In testimony whereof, I have signed my name to this specification.

H. STANLEY TIRRELL.